

Sept. 13, 1955

C. WRIGHT ET AL  
HEAT CONDUCTIVE MASTIC

2,717,839

Filed Nov. 9, 1951



Fig. 1



Fig. 2

Charles Wright  
Warren A. Hanson  
INVENTOR.

BY Robert M. Dunning  
ATTORNEY

# United States Patent Office

2,717,839

Patented Sept. 13, 1955

1

2,717,839

## HEAT CONDUCTIVE MASTIC

Charles Wright and Warren A. Hanson, St. Paul, Minn., assignors to Seeger Refrigerator Company, St. Paul, Minn.

Application November 9, 1951, Serial No. 255,700

4 Claims. (Cl. 106—285)

Our invention relates to an improvement in heat conductive mastic and deals particularly with a type of material used for securing a refrigerator coil to the liner of a refrigerator or freezer cabinet.

The instant application is a continuation-in-part of our nonforfeited co-pending application, Serial No. 73,098, filed January 27, 1949.

Freezer cabinets usually include an inner heat conductive liner and an outer shell separated and supported by insulation. A suitable mechanical refrigerating system is provided for cooling the space within the liner, this refrigerating system ordinarily circulating refrigerant through suitable evaporator coils either within the liner or attached thereto. In certain types of such freezers, metal coils are mechanically attached to the metallic liners of the cabinet and held in close contact with the sides and sometimes the bottoms thereof. Contact between the coils and the liner acts to conduct heat from the liner to the refrigerant within the coil. As the refrigerator coils are usually circular in cross section they can actually contact the surface of the liner only along a single line of contact. In order to increase the heat transfer from the liner to the coil, a beading of heat conductive mastic applied between the coil and the liner transfers heat through the mastic as well as through the actual line of contact between the coil and the liner. This mastic also serves as a heat transfer medium between the liner and the coil at points where the coil is slightly spaced from the liner, it being understood that it is difficult to hold the coil in contact with the liner throughout its entire length.

The present invention lies in the provision of a novel type of heat conductive mastic which has been found to provide superior thermo-conductivity. As any increase in the thermo-conductivity between the coil and the liner tends to increase the over-all operating efficiency of the freezer, the mastic thus produced tends to make the freezer more efficient than when other mastic is used.

A feature of the present invention lies in the use of a mastic between a refrigerant coil and a surface to be cooled which includes magnesium oxide combined with an oil. This combination provides better thermo-conductivity between the coil and the surface to be cooled than other mastic with which we are familiar, thereby increasing the efficiency of the freezer.

These and other objects and novel features of our invention will be more clearly and fully set forth in the following specification and claims.

In the drawings forming a part of our specification:

Figure 1 is a sectional view through a portion of a freezer wall showing the manner in which the coil is held in close contact with the walls of the liner.

Figure 2 is an enlarged sectional view through a coil and through a portion of the liner showing the manner in which the mastic acts to connect the coil and the heat conductive liner.

The freezer A illustrated in the accompanying drawings is only partially shown and the specific arrangement

2

illustrated is only indicative of one type of construction with which our invention may be used. The refrigerator A includes an outer casing 10 which is shown as having outer side wall panels such as 11 and a bottom panel 12. The side wall panels 11 are ordinarily rectangularly arranged, but may be cylindrical in form, or any other desired shape.

The refrigerator also includes an inner liner 13 which is usually formed of metal or other material of relatively high heat conductivity and which includes side walls such as 14 and a bottom wall 15. Insulation 16 is provided in the space between the liner bottom wall 15 and the casing bottom wall 12 and similar insulation 17 is provided between the liner side walls 14 and the casing side walls 11. In the specific arrangement illustrated the side walls 11 of the outer casing are provided with inturned marginal flanges 19, while the side walls 14 of the liner 13 are provided with outwardly turned flanges 20 which may extend substantially flush with the flanges 19. Suitable means 21 are provided for spacing and connecting the flanges 20 and 21, and a breaker strip 22 overlies the joint between the liner and the outer casing to serve as a closure therefore. In the particular arrangement illustrated the strip 22 is of plastic or similar material and is channel shaped in cross section to enclose a portion of the upper edge of the refrigerator.

The cabinet is usually closed by a door 23 which may be hinged to one of the side walls of the cabinet. The door 23 includes an outer sheathing 24 and an inner lining panel 25. The outer covering 24 may extend marginally toward the liner 25 and may terminate in an inwardly extending marginal flange 26 which may be spaced from the liner 25 by a suitable gasket 27. As previously stated this arrangement is only illustrated for the purpose of disclosing one type of construction with which our mastic may be used.

The evaporator coil 29 encircles the side walls 14 of the liner 13 and lies in contact therewith throughout as great a portion of its length as is practical. The evaporator coil 29 serves as a means containing refrigerant which is circulated through the coil by a suitable compressor. The details of the refrigerant circulating system have not been disclosed as they form no part of the present invention. The coil 29 may extend only about the side walls 14 of the freezer or may also underlie the bottom panel 15 of the liner as illustrated.

As best shown in Figure 2 of the drawings the evaporator coil 29 usually comprises an elongated metallic tube which is held in contact with the wall 14 or 15 of the freezer so as to provide a heat conductive joint therebetween. A generally triangular space is produced between each side of the tube or coil 29 and the liner wall. This generally triangular space is filled with mastic 30 so as to provide a good thermal contact between a relatively large area of the coil and the liner panel. If desired the mastic 30 can be applied on both sides of the line of contact between the coil and the liner rather than being merely on one side thereof as illustrated.

The mastic 30 is composed of magnesium oxide and an oil. However, as a preliminary to an understanding of the various oils that may be used in forming the mastic 30, it is to be noted that finished refining products may be generally grouped as follows:

I. Volatile products—liquefied gases and natural gasoline.

II. Light oils—gasolines, solvents, tractor fuel and kerosene.

III. Distillates—range oil, furnace distillates, diesel fuel and gas oil.

IV. Lubricating oil—motor, engine, machine, cylinder, spindle, gear, etc. oils.

V. Greases and waxes—paraffin wax, microcrystalline wax, petrolatum, salve bases and greases.

VI. Residues—fuel, coke, asphalt, carbon black, etc.

VII. Specialties—medicinal products, chemicals, insecticides, etc.

It is with the heavier and more viscous oils falling into group IV with which we are now concerned. These oils are listed below as follows:

| Name of Oil                | Degrees A. P. I. | Viscosity, Saybolt Universal Seconds @ 210° F. |
|----------------------------|------------------|------------------------------------------------|
| Motor, heavy               | 20-27            | 80-155                                         |
| Aircraft engine, heavy     | 23-25            | 100-145                                        |
| Transmission Oil, heaviest | 20-22            | 200-220                                        |
| Cylinder oils:             |                  |                                                |
| Light mineral              | 25-28            | 135-165                                        |
| Heavy mineral              | 20-26            | 175-220                                        |
| Light compounded           | 25-28            | 95-110                                         |
| Heavy compounded           | 20-26            | 175-220                                        |

As a specific example of the mastic which we have found to best suit the overall purposes of the present invention, we may cite the following:

*Example I*

58% by weight magnesium oxide  
42% by weight steam refined cylinder oil of 23-25 degrees A. P. I.

A second composition that is quite similar to Example I is presented below:

*Example II*

58% by weight magnesium oxide  
42% by weight cylinder oil of 23-25 degrees A. P. I. and approximately 200 S. U. secs.

The proportion of magnesium oxide used in the above cited example may be increased or decreased approximately 1% without greatly affecting the results and the percentage of oil may also be increased or decreased approximately 1%. With oil of the viscosity described above the mastic produced tends to become unduly soft and to run down the walls of the liner if the proportion of oil is increased more than approximately 1%. Similarly if the proportion of oil is decreased more than approximately 1%, the mastic becomes difficult to mix and to handle with ease. Oil of the particular viscosity mentioned provides a better heat transfer than oil of other viscosity in the mixture. Thus while the formula of the specific example mentioned may be varied without entirely losing the advantage of the combination, the above formula has been found to be advantageous over other proportions.

The viscosity of the oil used may be changed and a change in the viscosity of the oil acts to somewhat change the proportion of magnesium oxide which may be used in the combination. However, if a lighter or less viscous oil is used the mastic tends to become unduly soft at room temperatures and an increase in the viscosity tends to make a mastic which is slightly more difficult to mix and handle and does not appear to have as good heat conductive properties as the specific oil described. Similarly the oil need not be cylinder oil to produce advantageous results, although the particular oil mentioned has been found better than any other type of oil used. Thus the selection of the oil to produce best results appears important, as well as the viscosity thereof.

With reference to the particular type of oil, any of the oils set forth in the above presented list are deemed suitable, these listed oils having a gravity range of 20-28 degrees A. P. I. and a viscosity range of 80-220 S. U. secs. Actually, it is possible to employ other oils than those obtained from petroleum, such other oils including coal tar derivatives and shale oils of the above viscosity range. Still further, it is sometimes of advan-

tage to compound oils; cylinder oil, for instance, when compounded with from 5-7% of tallow adheres more closely to the metallic surfaces constituting the liner 13 and the coils 29. However, in general, compounding is practiced principally in order to meet viscosity specifications and therefore can be used to whatever extent is necessary to prevent the oil from running down the panel walls. A number of compounding substances are available, and it is believed that their respective characteristics are sufficiently well known for their proper use by those familiar with the oil refining art.

Magnesium oxide appears to have better heat conductive properties in the combination mentioned than other materials of a somewhat similar character and thus is believed specifically advantageous in the combination.

While the 58 to 42 percent ratio of magnesium oxide to oil is preferred, this ratio may be varied so that the magnesium oxide covers a range of from 52-66% with the remainder being oil. When 66% magnesium oxide is used, the less viscous oils of the preceding list may be best utilized, as in the following:

*Example III*

66% by weight magnesium oxide  
34% by weight heavy motor oil of 20-27 degrees A. P. I. and a viscosity of 80 to 155 S. U. seconds at 210° F.

When 52% magnesium oxide is used, the more viscous oils of the preceding list serve very well, as in the example below:

*Example IV*

52% by weight magnesium oxide  
48% by weight transmission oil of 20-22 degrees A. P. I. and 200-220 S. U. secs.

As before stated, the important thing is to produce a mastic of magnesium oxide and oil having a puttylike texture that will not permit the oil contained therein to separate out and run from the mastic at room temperatures. Of the examples presented, Example I has been found to be superior from an overall characteristic standpoint; i. e. it has been discovered from actual tests that it possesses all the factors necessary to produce a mastic for the particular purpose disclosed.

In accordance with the patent statutes, we have described the principles of construction and operation of our heat conductive mastic, and while we have endeavored to set forth the best embodiment thereof, we desire to have it understood that obvious changes may be made within the scope of the following claims without departing from the spirit of our invention.

We claim:

1. A heat conductive mastic consisting essentially of 52-66% by weight magnesium oxide and the remainder an oil, primarily mineral, having a viscosity range of from 80-220 Saybolt Universal seconds at 210° F.
2. A heat conductive mastic consisting essentially of substantially 58% by weight magnesium oxide and 42% by weight cylinder oil.
3. The composition described in claim 2 in which the cylinder oil has a gravity of from 23 to 25 degrees A. P. I.
4. A heat conductive mastic consisting essentially of substantially 58% by weight magnesium oxide and the remainder an oil selected from the class of heavy lubricating oils having a viscosity within the range of 80-220 Saybolt Universal seconds at 210° F.

References Cited in the file of this patent

UNITED STATES PATENTS

- |    |           |         |               |
|----|-----------|---------|---------------|
| 70 | 1,283,546 | Olson   | Nov. 5, 1918  |
|    | 1,619,534 | Olson   | Mar. 1, 1927  |
|    | 1,920,926 | Noonan  | Aug. 1, 1933  |
|    | 2,111,414 | Work    | Mar. 15, 1938 |
|    | 2,321,522 | Sands   | June 8, 1943  |
| 75 | 2,418,795 | Skolnik | Apr. 8, 1947  |
|    | 2,550,452 | Byrne   | Apr. 24, 1951 |